

[54] PROCESS FOR THE PRODUCTION OF A MULTICOLOR IMAGE BY IMAGE-WISE DYE DIFFUSION TRANSFER

[75] Inventors: **Wilhelmus Janssens, Aarschot; Daniël A. Claeys, Mortsel, both of Belgium**

[73] Assignee: **AGFA-Gevaert, N.V., Mortsel, Belgium**

[21] Appl. No.: **292,207**

[22] Filed: **Aug. 12, 1981**

[30] Foreign Application Priority Data

Sep. 30, 1980 [GB] United Kingdom ..... 8031504

[51] Int. Cl.<sup>3</sup> ..... G03C 5/54; G03C 1/40; G03C 7/00; G03C 1/10

[52] U.S. Cl. ..... 430/239; 430/214; 430/218; 430/223; 430/242

[58] Field of Search ..... 430/214, 218, 223, 239, 430/242, 487

[56] References Cited

U.S. PATENT DOCUMENTS

2,857,274 10/1958 Land et al. ..... 430/251  
3,335,009 8/1967 Rasch et al. ..... 430/489  
3,537,849 11/1970 Becker ..... 430/218  
3,630,730 12/1971 Stewart et al. ..... 430/218

3,698,898 10/1972 Grasshoff et al. ..... 430/219  
3,801,318 4/1974 Land et al. ..... 430/218  
4,139,379 2/1979 Chasman et al. ..... 430/223  
4,232,107 11/1980 Janssens ..... 430/218

Primary Examiner—Richard L. Schilling  
Attorney, Agent, or Firm—A. W. Breiner

[57] ABSTRACT

A process for the production of a multi-color dye image by dye diffusion transfer operating with a photographic multilayer multi-color material containing different non-diffusing dyes or dye precursor compounds that when contacted with an aqueous alkaline liquid remain immobile in an alkali-permeable colloid layer but are capable of being reduced by a developing agent at a rate slower than the reduction of image-wise developable silver halide and in reduced state under alkaline conditions are capable of releasing a diffusible dye or dye precursor moiety, and wherein as illustrated in the drawing dye images with higher color saturation are obtained by more extensive oxidation of developing agent in the image-wise photo-exposed area due to the use in the alkaline processing liquid of a silver halide solvent forming an alkali-soluble and reducible silver complex compound.

9 Claims, 1 Drawing Figure





**PROCESS FOR THE PRODUCTION OF A  
MULTICOLOR IMAGE BY IMAGE-WISE DYE  
DIFFUSION TRANSFER**

The present invention relates to a process for the production of a multicolour image by image-wise dye diffusion transfer.

Dye-diffusion transfer systems for the production of multicolour dye images operate with photosensitive silver halide materials and can be carried out in a number of ways. They are all based on the same principle, viz. the alteration in the mobility of a dye or dye-forming structural part of a compound controlled by the image-wise development of the silver halide to silver.

According to a first system a diffusible dye is produced image-wise by reaction of a particular initially immobile image-dye-providing compound with image-wise oxidized developing agent. Examples of such systems providing on development positive diffusion transfer dye images with an image-wise exposed direct-positive working silver halide emulsion material are described, e.g., in the U.K. Patent Specification No. 1,243,048 corresponding with the German Patent Specification No. 1,772,929, in the U.S. Pat. Nos. 3,227,550 and 3,628,952, and in the published U.S. Ser. No. B 351,673.

In one embodiment of the production of positive dye images said first system operates with a silver halide solvent and silver-precipitating layers, which contain development nuclei for obtaining therein through the silver complex diffusion transfer reversal process (DTR-process) a silver image and oxidized developing agent in correspondence with the non-photoexposed area as is described, e.g., in the published European Patent Application No. 0 003 376.

According to a second system a diffusible dye is produced image-wise by reaction of a particular initially immobile image-dye-providing compound with image-wise remaining non-oxidized developing agent. Examples of such systems providing positive diffusion transfer dye images with an image-wise exposed negative working silver halide emulsion material on development are described, e.g., in the U.S. Pat. Nos. 4,139,379 and 4,139,389, in the published European Patent Application No. 0 004 399, and in the European Patent Application No. 81 200303.6.

According to Research Disclosure 15511, published March 1977, a colour diffusion transfer process of the first system as exemplified in the U.S. Pat. Nos. 3,227,550 and 3,628,952, and in the German Patent Specification No. 1,772,929 is modified for the purpose of economizing on silver.

In said process an image-wise exposed and already developed colour photographic material is subjected to a second treatment with a developing bath containing a suitable silver halide solvent and optionally silver ions. The silver ions from the unexposed portions complexed with the silver solvent are reduced by physical development at the site of the already formed silver image, so without the aid of overall applied developing nuclei in special silver-precipitating layers. Thus in a photographic material with low silver content the silver image density becomes enhanced while simultaneously the developing agent is oxidized image-wise. Since according to the first mentioned dye diffusion transfer system the concentration of the oxidized developing agent defines the degree of dye-release colour images

with higher optical densities are obtained with less initially present silver halide. Indeed, according to said process the essential feature is to mobilize the silver halide that has not been exposed to use it in dissolved form as a silver complex compound to enhance by physical development the already obtained silver image in the exposed area.

It has been established experimentally that in a dye diffusion transfer process of said second system in multicolour image formation unwanted dye release takes place to some extent in the photo-exposed area of a photographic negative working multilayer multicolour silver halide emulsion material because unaffected, i.e. unoxidized, developing agent can diffuse from neighbouring layers into the area containing already developed silver halide. To make it explicitly clear a negative working emulsion yields on development a silver image in the photoexposed area.

**SUMMARY OF THE INVENTION**

It has been found now that when carrying out the development of said dye-releasing photographic multilayer multicolour material in the presence of a silver halide solvent capable of forming an alkali-soluble and reducible silver complex compound, said unwanted dye release from photoexposed area is diminished and even can be ruled out completely.

Thus, in accordance with the present invention a process for the production of a multicolour dye image by dye diffusion transfer is provided, comprising the steps of:

(1) image-wise multicolour photo-exposing a photographic multilayer multicolour material, which contains at least one developing agent and which is free from development nuclei for the silver complex diffusion transfer process and comprises a support carrying at least two differently spectrally sensitized alkali-permeable silver halide hydrophilic colloid emulsion layers each of which contains in operative contact therewith or therein a different non-diffusing dye or dye precursor compound that when contacted with an aqueous alkaline liquid remains immobile in an alkali-permeable colloid layer and is capable of being reduced by the said developing agent at a rate slower than the reduction of image-wise developable silver halide and in reduced state under alkaline conditions is capable of releasing a diffusible dye or dye precursor moiety, and

(2) applying an alkaline liquid to said photoexposed material, thus effecting development of the photoexposed material and image-wise diffusion-transfer therefrom of said diffusible dye or dye precursor moiety to a receptor layer, characterized in that said alkaline liquid during the development contains a silver halide solvent forming an alkali-soluble and reducible silver complex compound.

**DETAILED DESCRIPTION OF THE  
INVENTION**

The term "non-diffusing" used herein has the meaning commonly applied to the term in photography and denotes materials that in any practical application do not migrate or wander through organic colloid layers, e.g. gelatin, when permeated with an aqueous alkaline liquid. The same meaning is to be attached to the term "immobile".

The term "diffusible" as applied to the materials of this invention has the converse meaning and denotes materials having the property of diffusing effectively

through the colloid layers of the photographic elements with an aqueous alkaline liquid. "Mobile" has the same meaning.

By "operative contact" is meant that for producing diffusion transfer of an image-wise released dye or dye precursor compound on applying an alkaline processing liquid in the presence of a photographic silver halide developing agent, said compound releasing a dye or dye precursor can come into chemically reactive contact with unoxidized developing agent in an amount that is controlled by the image-wise developable silver halide of an image-wise photo-exposed silver halide emulsion layer.

The quoted terms are sufficiently known to those skilled in the art.

Suitable compounds releasing a dye or dye precursor for use according to the present invention are described in the U.S. Pat. Nos. 4,139,379 and 4,139,389, in the published European Patent Application No. 0 004 399 and in European Patent Application No. 81 200303.6, which documents have to be read in conjunction herewith.

An image-wise dye release by reaction with a non-oxidized developing agent acting as electron donor (ED-compound) proceeds e.g. according to the following reaction mechanism illustrated with simplified general formulae of quinonoid compounds (I):



4

quinone nucleus. Thus, said BEND-compounds used according to the present invention are ballasted compounds capable of undergoing an electron-accepting nucleophilic displacement reaction separating hereby in alkaline medium a diffusible dye or dye precursor moiety.

Other particularly suitable compounds releasing a dye or dye precursor for use according to the present invention are described in the published European Patent Application No. 0 004 399. In the latter Application quinone-type or quinonoid compounds are described, which compounds by reduction yield hydroquinone type compounds that through the action of alkali ( $\text{HO}^-$ ) are split into a ballasted quinone methide compound and a diffusible compound containing a dye moiety.

The image-wise dye release by reaction with a developing agent acting as electron donor (ED-compound) proceeds according to the following reaction mechanism illustrated with simplified general formulae of quinonoid compounds (I)<sup>1</sup>



The above BEND compounds and quinone-methide-yielding compounds are so-called IHR-compounds i.e. compounds of which the hydrolysability increases by reduction, wherein IHR is the acronym for "Increased Hydrolysis by Reduction". The above IHR-compounds release in reduced state under alkaline conditions a diffusible dye or dye precursor moiety.

According to one embodiment of the present invention the above process is carried out with a photographic material containing at least two differently spectrally sensitized silver halide emulsion layers and a different IHR-compound in operative contact with each silver halide emulsion layer. The IHR-compound comprises a dye-providing moiety, which includes a dye, a shifted dye or a dye precursor such as an oxichromic compound or a colour coupler.

In a preferred embodiment the process of the present invention is carried out with a photographic multilayer,

The dye compound (V) is released where the nucleophilic group, here the hydroxyl group of the hydroquinone, can attack the carbamate ester linkage. However, when the nucleophilic group is oxidized, which is the case in the quinone form, nucleophilic displacement is impossible. The compounds of the above formula (I) are referred to in said U.S. Pat. No. 4,139,379 as BEND-compounds wherein BEND is an acronym for Ballasted Electron-accepting Nucleophilic Displacement.

As is known in the art, "ballast" stands for ballasting group, which group makes the molecule immobile. The ballasting group may be present as a substituent on the

multicolour material, which comprises a layer containing a red-sensitive silver halide emulsion having in operative contact therewith an IHR-compound comprising a diffusible moiety providing a cyan image dye, a layer containing a green-sensitive silver halide emulsion having in operative contact therewith an IHR compound comprising a diffusible moiety providing a magenta image dye, and a layer containing a blue-sensitive silver halide emulsion having in operative contact therewith an IHR compound comprising a diffusible moiety providing a yellow image dye.

The moiety providing the image dye may be a pre-formed dye or a shifted dye. Dye materials of this type are well-known in the art and include azo dyes, azomethine (imine) dyes, anthraquinone dyes, alizarine dyes, merocyanine dyes, quinoline dyes, cyanine dyes and the like. As is known in the art, shifted dyes include those compounds whose light-absorption characteristics are shifted hypsochromically or bathochromically when subjected to a different environment such as a change in pH, a reaction with a material to form a complex, a tautomerization, reactions to change the pKa of the compound, a removal of a group such as a hydrolyzable acyl group connected to an atom of the chromophore as mentioned in Weyerts, U.S. Pat. No. 3,260,597 issued July 12, 1966, and the like. In certain embodiments the shifted dyes are highly preferred, especially those containing a hydrolyzable group on an atom affecting the chromophore resonance structure, since the compounds can be incorporated directly in a silver halide emulsion layer or even on the exposure side thereof without substantial reduction of the light that is effective in the exposure of the silver halide. After exposure the dye can be shifted to the appropriate colour such as, e.g., by hydrolytic removal of an acyl group to provide the respective image dye.

In another embodiment the IHR-compounds used in this invention contain an image dye-providing moiety, which is an image-dye precursor. The term "image-dye precursor" is understood to refer to those compounds that undergo reactions encountered in a photographic imaging system to produce an image dye such as colour couplers, oxichromic compounds, and the like.

When colour couplers are used they can be released in areas where no development occurs and can diffuse to an adjacent layer where they can be made to react with an oxidized colour developer such as an oxidized primary aromatic amine to form the image dye. Generally, the colour coupler and the colour developer are chosen so that the reaction product is immobile. Typical useful colour couplers include the pyrazolone couplers, pyrazolotriazole couplers, open-chain ketomethylene couplers, phenolic couplers and the like. Further reference to the description of appropriate couplers is found in U.S. Pat. No. 3,620,747 of John C. Marchant and Robert F. Motter, issued Nov. 16, 1971, which is incorporated herein by reference.

The compounds containing oxichromic moieties can be advantageously used in a photographic system since they are generally colourless materials because of the absence of an image-dye chromophore. Thus, they can be used directly in the photographic emulsion or on the exposure side, thereof without competitive absorption. Compounds of this type are those compounds that undergo chromogenic oxidation to form the respective image dye. The oxidation can be carried out by aerial oxidation, incorporation of oxidants into the photographic element or film unit, or use of an oxidant during

processing. Compounds of this type have been referred to in the art as leuco compounds, i.e. compounds that have no colour. Typical useful oxichromic compounds include leuco indoanilines, leuco indophenols, leuco anthraquinones and the like.

In the process of the present invention a silver halide developing agent is used that has sufficient reducing power to reduce photoexposed silver halide at a rate faster than in the reduction of the applied IHR compounds.

Photographic silver halide developing agents suitable for that purpose can be found by simple tests by using them in combination with an elected set of silver halide and IHR compound.

Typical useful silver halide developing agents applicable in the present invention include: hydroquinone compounds, 1-arylpyrazolidin-3-one compounds, pyrogallol and substituted pyrogallol compounds and ascorbic acid or mixtures thereof.

In a preferred embodiment the present process is carried out with a mixture of reducing agents one group of which is called electron donors (ED-compounds) and the other group is called electron-transfer agents (ETA-compounds). Generally, the electron-transfer agent is a compound that is a better silver halide reducing agent under the applied conditions of processing than the electron donor and, in those instances where the electron donor is incapable of, or substantially ineffective in developing the silver halide, the ETA-compound functions to develop the silver halide and provides a corresponding image-wise pattern of oxidized electron donor because the oxidized ETA-compound readily accepts electrons from the ED-compound.

The interlayer diffusion of the ED-compounds is effectively reduced by providing thereto a ballasting group so that they remain immobile in the layer unit wherein they have to transfer their electrons to the IHR compound associated therewith.

So, the ED-compound is preferably used in non-diffusible state in each silver halide emulsion layer containing a different non-diffusible dye or dye precursor. An example of such ED-compound as ascorbyl palmitate. Other ED-compounds are disclosed in U.S. Pat. No. 4,139,379 and in the published German Patent Application (DE-OS) No. 2,947,425. The ETA-compound on the contrary is preferably used as developing agent in diffusible state and is, e.g., incorporated in mobile form in (a) hydrophilic colloid layer(s) adjacent to one or more silver halide emulsion layers.

In this way the reactions are better separated in their desired sequence in that first the image-wise oxidation of the ETA-compound by the exposed silver halide starts, then the rapid electron transfer of oxidized ETA-compound to the ED-compound takes place, which compound being the less reactive compound where unaffected finally reacts with the IHR-compound to release the dye providing moiety.

Typically useful ETA-compounds include hydroquinone compounds such as hydroquinone, 2,5-dichlorohydroquinone, 2-chlorohydroquinone and the like; aminophenol compounds such as 4-aminophenol, N-methylaminophenol, 3-methyl-4-aminophenol, 3,5-dibromoaminophenol and the like; catechol compounds such as catechol, 4-cyclohexylcatechol, 3-methoxycatechol, 4-(N-octadecylamino)catechol and the like; phenylenediamine compounds such as N,N-diethyl-p-phenylenediamine, 3-methyl-N,N-diethyl-p-phenylenediamine, 3-methoxy-N-ethyl-ethoxy-p-

phenylenediamine, N,N,N',N'-tetramethyl-phenylenediamine and the like. In highly preferred embodiments, the ETA is a 3-pyrazolidinone compound such as 1-phenyl-3-pyrazolidinone, 1-phenyl-4,4-dimethyl-3-pyrazolidinone, 4-hydroxymethyl-4-methyl-1-phenyl-3-pyrazolidinone, 1-m-tolyl-3-pyrazolidinone, 1-p-tolyl-3-pyrazolidinone, 1-phenyl-4-methyl-3-pyrazolidinone, 1-phenyl-5-methyl-3-pyrazolidinone, 1-phenyl-4,4-bis-(hydroxymethyl)-3-pyrazolidinone, 1,4-dimethyl-3-pyrazolidinone, 4-methyl-3-pyrazolidinone, 4,4-dimethyl-3-pyrazolidinone, 1-(3-chlorophenyl)-4-methyl-3-pyrazolidinone, 1-(4-chlorophenyl)-4-methyl-3-pyrazolidinone, 1-(3-chlorophenyl)-3-pyrazolidinone, 1-(4-chlorophenyl)-3-pyrazolidinone, 1-(4-tolyl)-4-methyl-3-pyrazolidinone, 1-(2-tolyl)-4-methyl-3-pyrazolidinone, 1-(4-tolyl)-3-pyrazolidinone, 1-(3-tolyl)-3-pyrazolidinone, 1-(2-trifluoroethyl)-4,4-dimethyl-3-pyrazolidinone, 5-methyl-3-pyrazolidinone and the like. A combination of different ETA's such as those disclosed in U.S. Pat. No. 3,039,869 can also be employed. Such developing agents can be employed in the liquid processing composition or may be contained, at least in part, in any layer or layers of the photographic element or film unit such as the silver halide emulsion layers, the dye image-providing material layers, interlayers, image-receiving layer, etc. The particular ETA selected will, of course, depend on the particular electron donor and IHR-compound used in the process and the processing conditions for the particular photographic element.

Migration of non-oxidized developing agent, e.g. acting as ETA-compound, proceeds non-image-wise and will have an adverse effect on correct colour rendering when surplus developing agent remains unoxidized in the photoexposed area of a negative working emulsion layer. Therefore, according to the present invention said silver halide solvent is used to mobilize unexposed silver halide in complexed form for helping to neutralize (i.e. oxidize by physical development) migrated developing agent in the photoexposed area wherein unaffected developing agent (ETA-compound) should no longer be available for reacting with the IHR-compound directly or through the applied ED-compound.

The concentration of ED-compound in the photographic material may vary within a broad range but is, e.g., in the molar range of 1:2 to 4:1 with respect to the non-diffusing dye or dye precursor compound. The ETA-compound may be present in the alkaline aqueous liquid used in the development step, but is used preferably in diffusible form in non-photo-sensitive hydrophilic colloid layers adjacent to at least one silver halide emulsion layer. The concentration of the ETA-compound in the photographic material is preferably in the same molar range as wherein the ED-compound is applied.

#### BRIEF DESCRIPTION OF THE DRAWING

The invention is illustrated with a schematic drawing, which relates to a photographic multilayer multicolour material 1 exposed through a multicolour original 2 and processed in contact with a receptor material 3 for the transferred dyes.

In said multicolour material 1 element 4 represents a support, which is coated in successive order with

(1) a red-sensitive silver halide emulsion layer 5 containing a non-diffusing dye compound comprising a

5 diffusible moiety providing a cyan image dye and a non-diffusing ED-compound,

(2) a hydrophilic colloid interlayer 6, e.g. gelatin layer, containing a diffusible ETA-compound,

(3) a green-sensitive silver halide emulsion layer 7 containing a non-diffusing dye compound comprising a diffusible moiety providing a magenta image dye and a non-diffusing ED-compound,

10 (4) a hydrophilic colloid interlayer 8, e.g. gelatin layer containing a diffusible ETA-compound,

(5) a blue-sensitive silver halide emulsion layer 9 containing a non-diffusing dye compound comprising a diffusible moiety providing a yellow image dye and a non-diffusing ED-compound, and

15 (6) a protective hydrophilic colloid layer 10, e.g. gelatin layer, containing a diffusible ETA-compound.

The ED-compound is, e.g., ascorbyl palmitate corresponding to the following structural formula:



and the ETA-compound is e.g. 1-phenyl-3-pyrazolidinone.

The area of the original 2 transmitting blue light are indicated by the letter B, those transmitting green light by the letter G and those transmitting red light by the letter R. A silver image is developed in the photoexposed area of the red-, green- and blue-sensitive area respectively indicated by the hatched parts of these layers 5, 7 and 9. A cyan dye is released image-wise from the area indicated with C in layer 5. A magenta dye is released image-wise from the area indicated with M in layer 7. A yellow dye is released image-wise from the area indicated with Y in layer 9. The hydrophilic colloid layers 10, 8 and 6 contain a diffusible ETA-compound, which by diffusion arrives in the photo-exposed as well as in the non-photoexposed area of the silver halide emulsion layers. Where ETA-compound is not completely oxidized in the photoexposed area by the developable exposed silver halide, non-photoexposed silver halide of a neighbouring silver halide emulsion layer indicated with Δ is mobilized according to the present invention with silver halide solvent to become physically developed with simultaneous oxidation of ETA-compound at the site of already developed silver halide (hatched area). By this operation less ETA-compound already diffused in the photoexposed area is left unoxidized so that dye release in the present system, as is desired, cannot or substantially not take place from the photoexposed area by reaction between unoxidized ETA or ED-compound compound with dye releasing compound e.g. IHR-compound available there.

In the receptor material 3 in positive correspondence with the original 2, blue dye parts "b", green dye parts "g" and red dye parts "r" are formed. If the green image parts "g" are taken as an example, it is seen that these parts have to be built up solely by released yellow and cyan dye. When, however, magenta dye is released from the photoexposed silver halide emulsion layer area (hatched area of layer 7) a darkened i.e. less bright green image is obtained.

The more extensive developer exhaustion that according to the present invention takes place with the transferred silver complex in the photoexposed areas prevents dye release from the photoexposed areas so

that dye images with higher colour saturation, i.e. more bright colour images, are obtained.

As is known to those skilled in the art of silver halide photography, a considerable number of compounds form alkali-soluble complexes with silver ions. Among the many silver halide solvents may be mentioned thiosulphates, thiocyanates, thiosugars, thioetheracids e.g. HOOC—(CH<sub>2</sub>—S—CH<sub>2</sub>)<sub>3</sub>—COOH or an active methylene compound having the methylene group linked directly to sulphonyl groups as e.g. in H<sub>3</sub>C—SO<sub>2</sub>—CH<sub>2</sub>—SO<sub>2</sub>—CH<sub>3</sub>. Preferably used are, however, water-soluble thiosulphates (particularly alkali metal thiosulphate or ammonium thiosulphate).

According to one embodiment the silver halide solvent acting as silver-ion-complexing agent is applied in the alkaline aqueous liquid that is used in the development step. A useful concentration of silver halide solvent, e.g. sodium thiosulphate, in said liquid is in the range of 0.1 g to 40 g per liter.

According to a special embodiment the complexing agent is set free in the presence of alkali from a precursor compound present in the photographic material during development. Precursor compounds, which in the presence of alkali release a diffusible photographic reagent such as a silver halide solvent, are described in the U.S. Pat. No. 3,698,898. Such precursor compounds, which in the presence of alkali are capable of splitting off a silver halide solvent compound, correspond to the following general formula:



wherein:

X represents the atoms necessary to complete a benzene or naphthalene nucleus,

Y is hydroxy or a substituent that upon hydrolysis provides hydroxy,

PHOTO represents a silver halide solvent moiety, e.g. a —S—SO<sub>3</sub>M group wherein M is an alkali metal or onium group, e.g. ammonium group,

BALLAST is a ballasting group rendering said compound less diffusible in a water-permeated hydrophilic colloid layer than it would be without said group, and n is 1 or 2.

According to an embodiment said precursor compound is incorporated in the receiving layer of the receptor material wherefrom it can reach the contacting photoexposed photographic multilayer multicolour material upon alkaline treatment. According to another embodiment said precursor compound is incorporated in the photographic material, e.g. in the layer also containing diffusible developing agent (ETA-compound) and/or in the silver halide emulsion layers themselves. The rate of release of the silver halide solvent may be controlled by selection of the appropriate Y substituent, e.g. in the form of an ester group, which hydrolyses more or less rapidly. In the —CH<sub>2</sub>— group of the above general formula one or both of the hydrogen atoms may be substituted by a hydrocarbon group, e.g. an alkyl group such as methyl or ethyl.

The photosensitive silver halide present in a multi-layer multicolour silver halide photographic material used in the process of the present invention is e.g. a silver halide of the group of silver chloride, silver bro-

lide, silver bromoiodide, silver chlorobromoiodide and the like, or mixtures thereof. The emulsions may be coarse- or fine-grain and can be prepared by any of the well-known procedures, e.g., single-jet emulsions, double-jet emulsions. They may be Lippmann emulsions, ammoniacal emulsions, thiocyanate- or thioether-ripened emulsions such as those described in U.S. Pat. Nos. 2,222,264 of Adolph H. Nietz and Frederick J. Russell, issued Nov. 19, 1940; 3,320,069 of Bernard D. Illingsworth, issued May 16, 1967; and 3,271,157 of Clarence E. McBride, issued Sept. 6, 1966. Surface-image emulsions or internal-image emulsions may be used such as those described in U.S. Pat. Nos. 2,592,250 of Edward Philip Davey and Edward Bowes Knott, issued Apr. 8, 1952; 3,206,313 of Henry D. Porter, Thomas H. James and Wesley G. Lowe, issued Sept. 14, 1965; and 3,447,927 of Robert E. Bacon and Jean F. Barbier, issued June 3, 1969. The emulsions may be regular-grain emulsions such as the type described by Klein and Moisar in J. Photogr. Sci., Vol. 12, No. 5, September/October, 1964, pp. 242-251. If desired, mixtures of surface- and internal-image emulsions may be used as described in U.S. Pat. No. 2,996,382 of George W. Luckey and John C. Hoppe, issued Aug. 15, 1961.

Negative-type or direct-positive emulsions may be used such as those described in U.S. Pat. Nos. 2,184,013 of John A. Leermakers, issued Dec. 19, 1939; 2,541,472 of William B. Kendall and George D. Hill, issued Feb. 13, 1951; 3,367,778 of Robert W. Berriaman, issued Feb. 6, 1968; 3,501,307 of Bernard D. Illingsworth, issued Mar. 17, 1970; 2,563,785 of Charles F. Ives, issued Aug. 7, 1951; 2,456,953 of Edward Bowes Knott and Guy William Willis, issued Dec. 21, 1948; 2,861,885 of Edwin H. Land, issued Nov. 25, 1958; 3,761,276 of Francis John Evans, issued Sept. 25, 1973; 3,761,266 of Kirby Mitchell Milton, issued Sept. 25, 1973; 3,736,140 of Susan Starr Collier and Paul Brewster Gilman Jr., issued May 29, 1973; and 3,730,723 of Paul Brewster Gilman Jr., Ronald George Raleigh and Thaddeus Donald Koszelak, issued May 1, 1973; and United Kingdom Patent Specification No. 723,019 filed Feb. 5, 1952 by Gevaert Photo-Producten N.V.

The silver halide emulsions useful in our invention are well-known to those skilled in the art. More details about their composition, preparation and coating are described, e.g. in Product Licensing Index, Vol. 92, December 1971, publication 9232, p. 107-109.

Generally speaking, the silver halide emulsion layers in the invention comprise photosensitive silver halide dispersed in gelatin and are about 0.2 to 2  $\mu$ m thick. Preferably the dye image-providing materials are dispersed therein.

The support for the photographic elements used in this invention may be any material as long as it does not deleteriously affect the photographic properties of the film unit and is dimensionally stable. Typical flexible sheet materials are paper supports, e.g. coated at one or both sides with an  $\alpha$ -olefin polymer, e.g. polyethylene, or are film supports e.g. cellulose nitrate film, cellulose acetate film, poly(vinyl acetal) film, polystyrene film, poly(ethylene terephthalate) film, polycarbonate film, poly- $\alpha$ -olefins such as polyethylene and polypropylene film, and related films of resinous materials. The support is usually about 0.05 to 0.15 mm thick.

In a photographic material for use according to the invention and containing two or more silver halide emulsion layers, each silver halide emulsion layer con-

taining a dye image-providing material or having the dye image-providing material present in a contiguous layer is preferably separated from the other silver halide emulsion layer(s) in the film unit by (an) interlayer(s), including e.g. gelatin, calcium alginate, or any of the colloids disclosed in U.S. Pat. No. 3,384,483 of Richard W. Becker, issued May 21, 1968, polymeric materials such as polyvinylamides as disclosed in U.S. Pat. No. 3,421,892 of Lloyd D. Taylor, issued Jan. 14, 1969, or any of those disclosed in French Patent Specification No. 2,028,236 filed Jan. 13, 1970 by Polaroid Corporation or U.S. Pat. Nos. 2,992,104 of Howard C. Haas, issued July 11, 1961 and 3,427,158 of David P. Carlson and Jerome L. Reid, issued Feb. 11, 1969.

The interlayers are permeable to alkaline solutions, and are about 1 to 5  $\mu\text{m}$  thick. Of course these thicknesses are approximate only and may be modified according to the product desired.

According to an embodiment for correct spectral exposure of a multicolour dye diffusion transfer material for use according to the present invention, a water-permeable colloid interlayer dyed with a yellow non-diffusing dye is applied below the blue-sensitive silver halide emulsion layer containing a yellow dye-releasing compound and a water-permeable colloid interlayer dyed with a magenta non-diffusing dye is applied below the green-sensitive silver halide emulsion layer containing the magenta dye-releasing compound.

The image-receiving material used in this invention has the desired function of mordanting or otherwise fixing the dye images transferred from the photosensitive element. The particular material chosen will, of course, depend upon the dye to be mordanted. If acid dyes are to be mordanted, the image-receiving layer can be composed of, or contain basic polymeric mordants such as polymers or aminoguanidine derivatives of vinyl methyl ketone such as described in U.S. Pat. No. 2,882,156 of Louis M. Minsk, issued Apr. 14, 1959, and basic polymeric mordants and derivatives, e.g. poly-4-vinylpyridine, the 2-vinylpyridine polymer metho-p-toluene sulphonate and similar compounds described in U.S. Pat. No. 2,484,430 of Robert H. Sprague and Leslie G. Brooker, issued Oct. 11, 1949, the compounds described in the published German Patent Application No. 2,200,063 filed Jan. 11, 1971 by Agfa-Gevaert A. G. Suitable mordanting binders include, e.g. guanylhydrazone derivatives of acyl styrene polymers, as described, e.g., in published German Patent Specification No. 2,009,498 filed Feb. 28, 1970 by Agfa-Gevaert A. G. In general, however, other binders, e.g. gelatin, would be added to the last-mentioned mordanting binders. Effective mordanting compositions are long-chain quaternary ammonium or phosphonium compounds or tertiary sulphonium compounds, e.g. those described in U.S. Pat. Nos. 3,271,147 of Walter M. Bush and 3,271,148 of Keith E. Whitmore, both issued Sept. 6, 1966, and cetyltrimethyl-ammonium bromide. Certain metal salts and their hydroxides that form sparingly soluble compounds with the acid dyes may be used too. The dye mordants are dispersed in one of the usual hydrophilic binders in the image-receiving layer, e.g. in gelatin, polyvinylpyrrolidone or partly or completely hydrolysed cellulose esters.

Generally, good results are obtained when the image-receiving layer, which is preferably permeable to alkaline solutions, is transparent and about 4 to about 10  $\mu\text{m}$  thick. This thickness, of course, can be modified depending upon the result desired. The image-receiving

layer may also contain ultraviolet-absorbing materials to protect the mordanted dye images from fading, brightening agents such as the stilbenes, coumarins, triazines, oxazoles, dye stabilizers such as the chromanols, alkylphenols, etc.

According to a particular embodiment the photosensitive material is made suitable for in-camera processing. Therefor the receiving layer is integral with the photographic material and is arranged in water-permeable relationship with the silver halide hydrophilic colloid emulsion layers. For that purpose the photosensitive silver halide emulsion layers are normally negative-working and applied to the same support as the receptor layer so as to form an integral combination of light-sensitive layer(s) and a non light-sensitive layer receiver element preferably with an opaque layer, which is alkali-permeable, reflective to light and located between the receptor layer and the silver halide emulsion layer(s). In a process using such material the alkaline processing composition may be applied between the outer photosensitive layer of the photographic element and a cover sheet, which may be transparent and superposed before exposure.

To form the opaque layer an opacifying agent can be applied from a processing composition. Examples of opacifying agents include carbon black, barium sulphate, zinc oxide, barium stearate, silicates, alumina, zirconium oxide, zirconium acetyl acetate, sodium zirconium sulphate, kaolin, mica, titanium dioxide, organic dyes such as indicator dyes, nigrisines, or mixtures thereof in widely varying amounts depending upon the degree of opacity desired. In general, the concentration of opacifying agent should be sufficient to prevent further exposure of the film unit's silver halide emulsion or emulsions by ambient actinic radiation through the layer of processing composition, either by direct exposure through a support or by light piping from the edge of the element. For example, carbon black or titanium dioxide will generally provide sufficient opacity when they are present in the processing solution in an amount of from about 5 to 40% by weight. After the processing solution and opacifying agent have been distributed into the film unit, processing may take place out of the camera in the presence of actinic radiation in view of the fact that the silver halide emulsion(s) of the laminate is (are) appropriately protected against incident radiation, at one major surface by the opaque processing composition and at the remaining major surface by the opaque layer that is permeable to alkaline solutions. In certain embodiments, ballasted indicator dyes or dye precursors can be incorporated in a layer on the exposure side of the photosensitive layers; the indicator dye is preferably transparent during exposure and becomes opaque when contacted with the processing composition. Opaque binding tapes can also be used to prevent edge leakage of actinic radiation incident on the silver halide emulsion.

When titanium dioxide or other white pigments are employed as the opacifying agent in the processing composition, it may also be desirable to employ in co-operative relationship therewith a pH-sensitive opacifying dye such as a phthalein dye. Such dyes are light-absorbing or coloured at the pH at which image formation is effected and colourless or not light-absorbing at a lower pH. Other details concerning these opacifying dyes are described in French Patent Specification No. 2,026,927 filed Dec. 22, 1969 by Polaroid Corporation.

The substantially opaque, light-reflective layer, which is permeable to alkaline solutions, in the receiver part of integral film units suited for use in the present invention can generally comprise any opacifier dispersed in a binder as long as it has the desired properties. Particularly desirable are white light-reflective layers since they would be esthetically pleasing backgrounds on which to view a transferred dye image and would also possess the optical properties desired for reflection of incident radiation. Suitable opacifying agents include, as already mentioned with respect to the processing composition, titanium dioxide, barium sulphate, zinc oxide, barium stearate, silver flake, silicates, alumina, zirconium oxide, zirconium acetyl acetate, sodium zirconium sulphate, kaolin, mica, or mixtures thereof in widely varying amounts depending upon the degree of opacity desired. The opacifying agents may be dispersed in any binder such as an alkaline solution-permeable polymeric matrix such as, for example, gelatin, polyvinyl alcohol, and the like. Britthening agents such as the stilbenes, coumarins, triazines and oxazolines may also be added to the light-reflective layer, if desired. When it is desired to increase the opacifying capacity of the light-reflective layer, dark-coloured opacifying agents may be added to it, e.g., carbon black, 20 nigrosine dyes, etc. Another technique to increase the opacifying capacity of the light-reflective layer is to employ a separate opaque layer underneath it comprising, e.g., carbon black, nigrosine dyes, etc., dispersed in a polymeric matrix that is permeable to alkaline solutions such as, e.g., gelatin, polyvinyl alcohol, and the like. Such an opaque layer should generally have a density of at least 4 and preferably greater than 7 and should be substantially opaque to actinic radiation. The opaque layer may also be combined with a developer 30 scavenger layer if one is present. The light-reflective and opaque layers are generally 0.025 to 0.15 mm in thickness, although they can be varied depending upon the opacifying agent employed, the degree of opacity desired, etc.

Use of pH-lowering material in the dye-image-receiving element of an integral film unit for use according to the invention usually increase the stability of the transferred image. Generally, the pH-lowering material will effect a reduction of the pH of the image layer from about 13 or 14 to at least 11 and preferably 5-8 within a short time after imbibition. For example, polymeric acids as disclosed in U.S. Pat. No. 3,362,819 of Edwin H. Land, issued Jan. 9, 1968 or solid acids or metallic salts, e.g. zinc acetate, zinc sulphate, magnesium acetate, etc., as disclosed in U.S. Pat. No. 2,584,030 of Edwin H. Land, issued Jan. 29, 1952, may be employed with good results. Such pH-lowering materials reduce the pH of the film unit after development to terminate development and substantially reduce further dye transfer and thus stabilize the dye image.

An inert timing or spacer layer may be employed in practice over the pH-lowering layer, which "times" or controls the pH reduction depending on the rate at which alkali diffuses through the inert spacer layer. Examples of such timing layers include gelatin, polyvinyl alcohol or any of the colloids disclosed in U.S. Pat. No. 3,455,686 of Leonard C. Farney, Howard G. Rogers and Richard W. Young, issued July 15, 1969. The timing layer may be effective in evening out the various reaction rates over a wide range of temperatures, e.g., premature pH reduction is prevented when imbibition is effected at temperatures above room temperature, e.g.

at 35° to 37° C. The timing layer is usually about 2.5  $\mu$ m to about 18  $\mu$ m thick. Especially good results are obtained when the timing layer comprises a hydrolysable polymer or a mixture of such polymers that are slowly hydrolysed by the processing composition. Examples of such hydrolysable polymers include polyvinyl acetate, polyamides and cellulose esters.

An alkaline processing composition employed in this invention may be a conventional aqueous solution of an alkaline material, e.g., sodium hydroxide, sodium carbonate or an amine such as diethylamine. Independent from the use of the silver halide solvent or in admixture therewith improved dye densities are obtained in the dye diffusion transfer process applying IHR-compounds when the alkaline processing liquid contains a saturated, aliphatic or alicyclic amino alcohol having from 2 to 10 carbon atoms and at least two hydroxy groups. Particularly high dye densities are obtained when using in said processing liquid triisopropanolamine. Other suitable dye density improving solvents, optionally used in admixture, are dimethylformamide, N-methyl-2-pyrrolidinone and an aliphatic or cycloaliphatic hydroxy-compound being e.g. a mono-alcohol, diol or triol that is not completely miscible with water at 20° C. Preferred examples thereof are n-butanol, isobutanol, 2,2-diethyl-propane-1,3-diol, 1-phenylethane-1,2-diol (styrene glycol), 2,2,4,4-tetramethylbutane-1,3-diol, 2-ethyl-hexane-1,3-diol and 1,4-cyclohexane-dimethanol.

Preferably the pH of the processing composition is at least 11. The processing composition does not have to contain the above defined silver halide solvent compound when the latter is already contained in a silver halide solvent precursor compound applied in the photographic material and/or receptor material.

According to one embodiment the alkaline processing liquid contains a diffusible developing agent e.g. ascorbic acid or a 3-pyrazolidinone developing agent such as 1-phenyl-4-methyl-3-pyrazolidinone serving e.g. as ETA-compound for effecting the reduction of the exposed and complexed silver halide.

The alkaline processing composition employed in this invention may also contain a desensitizing agent such as methylene blue, nitro-substituted heterocyclic compounds, 4,4'-bipyridinium salts, etc., to insure that the photosensitive element is not further exposed after it is removed from the camera for processing.

The solution also preferably contains a viscosity-increasing compound such as a high-molecular-weight polymer, e.g. a water-soluble ether inert to alkaline solutions such as hydroxyethylcellulose or alkali metal salts of carboxymethylcellulose such as sodium carboxymethylcellulose. A concentration of viscosity-increasing compound of about 1 to about 5% by weight of the processing composition is preferred. It will impart thereto a viscosity of about 100 mPa.s to about 200,000 mPa.s.

Processing of separable photographic material and dye-receiving material may proceed in a tray developing unit as is present, e.g. in an ordinary silver complex diffusion transfer (DTR) apparatus in which contacting with the separate dye image-receiving material is effected after a sufficient absorption of processing liquid by the photographic material has taken place. A suitable apparatus for said purpose is the COPYPROOF CP 38 (trade name) DTR-developing apparatus. COPYPROOF is a trade name of Agfa-Gevaert, Antwerp-/Leverkusen.

According to the other embodiments wherein the receptor layer is integral with the photosensitive layer(s) the processing liquid is applied e.g. from a rupturable container or by spraying.

The rupturable container may be of the type disclosed in U.S. Pat. Nos. 2,543,181 of Edwin H. Land, issued Feb. 27, 1951; 2,643,886 of Ulrich L. di Ghilini, issued June 30, 1953; 2,653,732 of Edwin H. Land, issued Sept. 29, 1953; 2,723,051 of William J. McCune Jr., issued Nov. 8, 1955; 3,056,492 and 3,056,491, both of 10 John E. Campbell, issued Oct. 2, 1962; and 3,152,515 of Edwin H. Land, issued Oct. 13, 1964. In general such containers comprise a rectangular sheet of fluid- and air-impervious material folded longitudinally upon itself to form two walls that are sealed to one another along 15 their longitudinal and end margins to form a cavity in which processing solution is contained.

While the alkaline processing composition used in this invention can be employed in a rupturable container, as described previously, to facilitate conveniently the introduction of processing composition into the film unit, other means of discharging processing composition within the film unit could also be employed, e.g., means injecting processing solution with communicating members similar to hypodermic syringes, which are attached either to a camera or camera cartridge, as described in U.S. Pat. No. 3,352,674 of Donald M. Harvey, issued Nov. 14, 1967.

The main aspect of the present invention is the use of silver halide solvent in a diffusion transfer system operating with IHR-type-compounds from which by reduction and in alkaline medium a dye is released as photographically useful fragment. This is the reason why mainly reference is made to colour providing compounds. The invention, however, is not at all limited to 30 this aspect and it should be kept in mind that for various other purposes other photographically useful fragments may be present in these compounds instead of dyes or dye precursors.

The following example further illustrates the invention. All percentages and ratios are by weight, unless otherwise mentioned.

#### EXAMPLE

A subbed water-resistant paper support consisting of 45 a paper sheet of 110 g/sq.m coated at both sides with a polyethylene stratum of 15 g/sq.m was treated with a corona discharge and thereupon coated in the mentioned order with the following layers:

50

(1) an alkali-permeable colloid layer containing after drying per sq.m:

|                                                                  |         |
|------------------------------------------------------------------|---------|
| gelatin                                                          | 0.940 g |
| cyan dye-providing quinonoid compound C <sub>1</sub>             | 0.230 g |
| (applied from a dispersion prepared as described hereinafter)    |         |
| silver chloride                                                  | 0.380 g |
| (applied from a red-sensitized gelatin-silver chloride emulsion) |         |
| 2,5-bis(1',1',3',3'-tetramethylbutyl)-hydroquinone               | 0.050 g |

55

60

-continued

|                                                                                                        |         |
|--------------------------------------------------------------------------------------------------------|---------|
| (2) an interlayer containing per sq.m:                                                                 |         |
| gelatin                                                                                                | 1.028 g |
| 1-phenyl-4-methyl-3-pyrazolidinone (added from a dispersion prepared as described hereinafter)         | 0.105 g |
| 2-acetyl-5-octadecyl(2)-hydroquinone as magenta filtering dye                                          | 0.090 g |
| Pigment Red 146 (C.I. 11,000)                                                                          | 0.910 g |
| (3) an alkali-permeable colloid layer containing per sq.m:                                             |         |
| gelatin                                                                                                | 1.040 g |
| magenta dye-providing quinonoid compound M <sub>1</sub>                                                | 0.184 g |
| (applied from a dispersion prepared as described hereinafter)                                          |         |
| 2,5-bis(1',1',3',3'-tetramethylbutyl)-hydroquinone                                                     | 0.045 g |
| silver chloride                                                                                        | 0.374 g |
| (applied from a green-sensitized gelatin-silver chloride emulsion)                                     |         |
| (4) an interlayer containing per sq.m:                                                                 |         |
| gelatin                                                                                                | 1.000 g |
| 1-phenyl-4-methyl-3-pyrazolidinone                                                                     | 0.102 g |
| 2-acetyl-5-octadecyl(2)-hydroquinone as yellow filtering dye                                           | 0.087 g |
| Pigment Yellow 83 (C.I. 20,000)                                                                        | 1.085 g |
| (5) an alkali-permeable colloid layer containing per sq.m:                                             |         |
| gelatin                                                                                                | 1.800 g |
| yellow dye-providing quinonoid compound Y <sub>1</sub>                                                 | 0.407 g |
| (applied from a dispersion as described hereinafter)                                                   |         |
| ascorbyl palmitate                                                                                     | 0.212 g |
| (added from a dispersion prepared as described hereinafter)                                            |         |
| silver chloride                                                                                        | 0.395 g |
| (applied from a blue-sensitive gelatin-silver chloride emulsion)                                       |         |
| (6) a protective layer containing per sq.m:                                                            |         |
| gelatin                                                                                                | 1.42 g  |
| 1-phenyl-4-methyl-3-pyrazolidinone-Preparation of the dispersion of 1-phenyl-4-methyl-3-pyrazolidinone | 0.105 g |

The preparation proceeded by sand-milling the following ingredients:

|                                              |        |
|----------------------------------------------|--------|
| gelatin                                      | 40 g   |
| 1-phenyl-4-methyl-3-pyrazolidinone           |        |
| 40% aqueous solution of LOMAR D (trade name) | 10 ml  |
| distilled water                              | 850 ml |

(LOMAR D is a trade name of Nopco Chemical Company, Newark, N.J., U.S.A. for a naphthalene sulphonate condensate, formaldehyde being used in the condensation reaction).

#### Preparation of the dispersion of ascorbyl palmitate

50 g of ascorbyl palmitate were first dissolved in 450 ml of ethanol forming solution A.

A solution of 125 g of gelatin in 1975 ml of distilled water was prepared and added to a solution containing 4.8 g of sodium hydroxide, 0.2 ml of n-octylalcohol and 95 ml of distilled water so as to form solution B. Thereupon solution A was thoroughly mixed with solution B.

#### Preparation of the dispersion of yellow dye-providing compound Y<sub>1</sub>

compound Y<sub>1</sub> prepared as described hereinafter and in the European Pat. Appl. No. 81 200303.6 as compound VII and having the structural formula:

-continued

|                                                                                                                                                                                                     |                                                                                                                             |
|-----------------------------------------------------------------------------------------------------------------------------------------------------------------------------------------------------|-----------------------------------------------------------------------------------------------------------------------------|
| <br>gelatin<br>N-methyl-2-pyrrolidinone<br>10% aqueous solution of MARLON A-396<br>(trade name)<br>distilled water | <br>20 g<br>50 g<br>20 g<br>20 ml<br>625 g |
|                                                                                                                                                                                                     |                                                                                                                             |
|                                                                                                                                                                                                     |                                                                                                                             |
|                                                                                                                                                                                                     |                                                                                                                             |
|                                                                                                                                                                                                     |                                                                                                                             |

Compound Y<sub>1</sub> was first dissolved in ethylacetate and added whilst vigorously stirring to the gelatin dissolved in the indicated amount of water. Thereupon the ethylacetate was removed by evaporation under reduced pressure.

MARLON A-396 is a trade name of Chemische

20 Preparation of the dispersion of magenta dye-providing compound M<sub>1</sub>

The preparation proceeded analogously to the preparation of the dispersion of compound Y<sub>1</sub> but wherein the following ingredients were used:

compound M<sub>1</sub> prepared as described hereinafter and in the European Pat. Appl. No. 81 200303.6 as compound VI and having the following structural formula:

|                                                                                                                                                                                 |                                                                                                                         |
|---------------------------------------------------------------------------------------------------------------------------------------------------------------------------------|-------------------------------------------------------------------------------------------------------------------------|
| <br>gelatin<br>10% aqueous solution of MARLON A-396<br>(trade name)<br>distilled water up to | <br>10 g<br>25 g<br>10 ml<br>1000 g |
|                                                                                                                                                                                 |                                                                                                                         |
|                                                                                                                                                                                 |                                                                                                                         |
|                                                                                                                                                                                 |                                                                                                                         |

Werke Hüls AG Marl/Westfalen, W. Germany for a wetting agent having the formula:



Preparation of the dispersion of cyan dye-providing compound C<sub>1</sub>

45 The preparation proceeded analogously to the preparation of the dispersion of compound Y<sub>1</sub> but wherein the following ingredients were used:

compound C<sub>1</sub> prepared analogously to the quinone derivative of compound 39 of European Pat. Appl. 0 004 399 and having the following structural formula:

|                                                                                                                                                                                 |                                                                                                                         |
|---------------------------------------------------------------------------------------------------------------------------------------------------------------------------------|-------------------------------------------------------------------------------------------------------------------------|
| <br>gelatin<br>10% aqueous solution of MARLON A-396<br>(trade name)<br>distilled water up to | <br>15 g<br>225 g<br>15 ml<br>300 g |
|                                                                                                                                                                                 |                                                                                                                         |
|                                                                                                                                                                                 |                                                                                                                         |
|                                                                                                                                                                                 |                                                                                                                         |

wherein R is C<sub>10</sub>-C<sub>13</sub> n-alkyl.

Exposure and processing

A sheet of the obtained photographic material was exposed through a green light-transmitting filter covered with a grey wedge having a constant 0.1 and there-

upon contacted with the receptor material described hereinafter in the COPYPROOF CP 38 (trade name) diffusion transfer processing apparatus containing in its tray an aqueous solution comprising per liter:

|                                                          |         |
|----------------------------------------------------------|---------|
| sodium hydroxide                                         | 25 g    |
| sodium orthophosphate                                    | 15 g    |
| trisopropanolamine                                       | 80 ml   |
| potassium bromide                                        | 1 g     |
| 1% ethanolic solution of 1-phenyl-2-tetrazoline-5-thione | 5 ml    |
| paraformaldehyde                                         | 2 g     |
| distilled water up to                                    | 1000 ml |

As indicated in the Tables 1 to 3 increasing amounts of silver halide solvents were added to said solution to check their influence on colour rendition.

#### COMPOSITION OF THE RECEPTOR MATERIAL

To the same support as described for the above light-sensitive material a coating having the following composition was applied per sq.m:

|                                          |     |
|------------------------------------------|-----|
| gelatin                                  | 5 g |
| triphenyl-n-hexadecylphosphonium bromide | 2 g |

#### Measurements

The blue, green and red absorption values of the green part image obtained with these modified solutions and a blank were measured behind Kodak Wratten filters Blue No. 47, Green No. 58 and Red No. 25 with a Macbeth (trade name) densitometer RD-100 R.

The above Wratten filters manufactured by The Eastman Kodak Company have transmission curves as represented in Handbook of Chemistry and Physics, 56th Edition, Editor Robert C. Weast—CRC Press 18901 Cranwoord Parkway, Cleveland, Ohio 44128 USA p. E-241 and E-240.

TABLE 1

| Added amount of<br>Na <sub>2</sub> S <sub>2</sub> O <sub>3</sub> in g/l | Relative absorption values<br>measured behind filters |       |     |
|-------------------------------------------------------------------------|-------------------------------------------------------|-------|-----|
|                                                                         | blue                                                  | green | red |
| —                                                                       | 114                                                   | 85    | 138 |
| 0.05                                                                    | 113                                                   | 84    | 138 |
| 0.10                                                                    | 107                                                   | 73    | 138 |
| 0.20                                                                    | 104                                                   | 70    | 138 |
| 0.50                                                                    | 100                                                   | 59    | 138 |
| 1.00                                                                    | 93                                                    | 52    | 138 |
| 2.00                                                                    | 95                                                    | 50    | 138 |
| 5.00                                                                    | 82                                                    | 48    | 138 |
| 10.00                                                                   | 85                                                    | 48    | 138 |
| 20.00                                                                   | 85                                                    | 48    | 138 |
| 40.00                                                                   | 95                                                    | 48    | 139 |

The lower the absorption of green light, the more brilliant the green image parts are. The absorption of blue and red light remains high with increasing amounts of silver halide solvent.

In the following Tables 2 and 3 the relative absorption values obtained with processing solution containing increasing amounts of  $\text{CH}_3\text{—SO}_2\text{—CH}_2\text{—SO}_2\text{—CH}_3$  and KSCN respectively as silver halide solvents are presented.

TABLE 2

| 5  | Added amount of<br>$\text{CH}_3\text{—SO}_2\text{—CH}_2\text{—SO}_2\text{—CH}_3$<br>in g/l | Relative absorption values<br>measured behind filters |       |     |
|----|--------------------------------------------------------------------------------------------|-------------------------------------------------------|-------|-----|
|    |                                                                                            | blue                                                  | green | red |
| —  | 0                                                                                          | 117                                                   | 85    | 130 |
| —  | 5                                                                                          | 110                                                   | 81    | 130 |
| —  | 10                                                                                         | 91                                                    | 48    | 130 |
| 10 | 20                                                                                         | 75                                                    | 49    | 130 |
| —  | 40                                                                                         | 60                                                    | 47    | 130 |

TABLE 3

| 15 | Added amount of<br>KSCN in g/l | Relative absorption values<br>measured behind filters |       |     |
|----|--------------------------------|-------------------------------------------------------|-------|-----|
|    |                                | blue                                                  | green | red |
| —  | 0                              | 117                                                   | 85    | 130 |
| —  | 2                              | 105                                                   | 73    | 130 |
| —  | 5                              | 91                                                    | 63    | 130 |
| —  | 10                             | 69                                                    | 45    | 130 |

#### PREPARATION OF COMPOUND M1 (COMPOUND VI)—FIRST MODE

##### (a) 2-Acetyl-5-methyl-hydroquinone (VIa)

496 g (4 mole) of methylhydroquinone and 512 ml of acetic acid were heated at 80° C. with stirring. Boron trifluoride gas was bubbled through whereby the reaction temperature reached 120° C. Stirring was then continued and the reaction temperature kept at 120° C. for 1 h. Whilst vigorous stirring the reaction mixture was poured into 6 l of ice-water containing 1 kg of sodium acetate. Stirring was continued for 12 h whereupon the precipitate formed was filtered off, first washed by stirring in water containing some sodium carbonate and then with pure water, and finally dried. Purification proceeded by extraction with CLAIRSOL 300 (trade name). Yield: 400 g. Melting point: 144°–146° C.

##### (b) 2-Acetyl-4-p-hexadecyloxyphenyl-5-methyl-hydroquinone (VIb)

166 g (1 mole) of compound VIa were dissolved in 4 l of methylene chloride. Then 500 g of precipitated manganese(IV) dioxide and 500 g of sodium sulphate were added with stirring. The reaction mixture was refluxed with stirring for 90 min and filtered through a layer of sodium sulphate. To the filtrate 310 g (0.975 mole) of n-hexadecyloxybenzene were added and stirring was continued till complete dissolution. The solution was cooled just below 2° C. with stirring and 500 ml of trifluoro acetic acid were dropwise added such that the temperature did not rise above 5° C. After a further stirring period of 1 h, still 300 g of manganese(IV) dioxide were added. Stirring was continued for 2 h. The precipitate of manganese(IV) dioxide was separated by suction and the filtrate concentrated to 1 l in a rotary evaporator. The concentrated filtrate was diluted with 2.5 l of ethyl acetate and 2.5 l of water, and treated with 1 kg of sodium hydrosulphite.

After being stirred for 15 min the organic liquid layer was separated, washed first with 2.5 l of water containing 140 g of sodium hydrogen carbonate and subsequently twice with 2 l of 15% by weight aqueous sodium chloride solution and dried with sodium sulphate.

The solid product was obtained by evaporating the volatile solvent in a rotary evaporator. Recrystalliza-

tion from 1.8 l of ethanol yielded 306 g of compound VIb. Melting point: 68° C.

(c)

2-(1-Hydroxyethyl)-3-p-hexadecyloxyphenyl-5-methylhydroquinone (VIc)

96.5 g of compound VIb dissolved in 600 ml of anhydrous ethanol were reduced at 70°-75° C. under a hydrogen pressure of 105 kg/sq.cm in the presence of Raney-nickel for 3 h.

The catalyst was removed by filtering and the filtrate cooled in ice. The precipitate formed was suction-filtered, washed twice with cold ethanol and dried under reduced pressure. Yield: 81.6 g. Melting point: 75° C. (structure confirmed by NMR).

(d) Hydroquinone form of compound M1 (VIId)

42.5 g of compound Q (prepared as hereinafter), 5 g of sodium acetate, 750 ml of acetic acid and 500 ml of water were dissolved at 60° C. forming solution A.

24.2 g of compound VIc were dissolved at 50° C. in 200 ml of acetic acid and added to solution A. The reaction mixture was stirred at 60° C. for 12 h. After cooling, the precipitate was filtered with suction, washed with a mixture of methanol/water (1:1 by volume) and dried. Yield: 47.5 g.

(e) Compound M1 (VI)

47.5 g of compound VIId were dissolved at 60° C. in 550 ml of ethylene glycol monomethyl ether. Then 8 g of p-benzoquinone were added and the reaction mixture was stirred at 60° C. for 1 h. After cooling to 40° C. the reaction mixture was poured with stirring into 1.5 l of water whereto 10 ml of concentrated hydrochloric acid were added. The formed precipitate was suction-filtered, washed with a mixture of methanol/water (1:1 by volume) dried and purified by preparative column chromatography on silica gel by means of a mixture of methylene chloride/ethyl acetate (90/10) as the eluent. Yield: 25 g. Melting point (unsharp): 100° C.

#### PREPARATION OF COMPOUND M1—SECOND MODE

(f)

2-(1-p-aminophenylsulphonylethyl)-3-p-hexadecyloxyphenyl-5-methyl-benzoquinone (VIIf)

51 g of p-aminobenzene-sulphinic acid and 121 g of compound VIc were stirred at 60° C. in a mixture of 1500 ml of acetic acid and 150 ml of water. To the mixture 15 ml of concentrated sulphuric acid were added at 60° C. and stirring was continued for 15 min. Oxidation of the hydroquinone proceeded by adding 230 ml of an aqueous iron(III)chloride solution (3.5 moles per liter) and stirring at 60° C. for 1 h. Thereupon 1500 ml of water were added to the reaction mixture at room temperature, and the precipitate was separated by suction-filtering and washed with water.

After recrystallization from benzine 64 g of compound VIIf were obtained. Melting point: 124° C.

(g) Compound M1

12.4 g of compound VIIf and 9.9 g of compound P (prepared as hereinafter) were stirred at 20° C. in a mixture of 150 ml of methylene chloride and 3 ml of pyridine for 90 min.

The formed precipitate was separated by suction-filtering and washed with methylene chloride. The filtrates were concentrated to dryness and the residue

purified by preparative column chromatography under pressure on silicagel as the adsorbent and by means of a mixture of methylene chloride/ethyl acetate (85/15 by volume) as an eluent. Yield: 5.4 g.

#### PREPARATION OF COMPOUND Y1 (COMPOUND VII)

(a) Hydroquinone form of compound Y1 (VIIa)

10 208 g of compound 1e prepared as described in the published European patent publication No. 0.004.399, 20 g of sodium acetate, 1.7 l of acetic acid and 1 l of water were stirred at 60° C. To the obtained mixture 96.8 g of compound VIc dissolved at 50° C. in 600 ml of acetic acid were added.

15 The reaction mixture was kept at 60° C. for 6 h. Thereupon the reaction mixture was cooled and the formed precipitate was suction-filtered, washed with a mixture of methanol/water 1:1 by volume and dried.

20 Crystallization proceeded by dissolving the product at 80° C. in 1 l of ethylene glycol monomethyl ether, hot filtering and heating again to 80° C. After the addition of 100 ml of water and stirring, the mixture was cooled.

25 The obtained precipitate was suction-filtered and washed with methanol. Yield: 98.5 g. Melting point: 138° C.

(b) Compound Y1 (VII)

30 98.5 g of compound VIIa were dissolved in 1 l of ethylene glycol monomethyl ether and 15 g of p-benzoquinone were added at 60° C. The reaction mixture was stirred at 60° C. for 1 h and cooled to 30° C. The precipitate formed was suction-filtered, washed with a mixture of methanol/water 1:1 by volume and dried. Yield: 92.5 g. Melting point: 139° C.

(a)

40 1-methylsulphonylamino-4-(2-cyanophenyl-azo)-7-sulphonaphthalene

To 600 ml of pyridine 223 g (1 mole) of 1-amino-7-sulpho-naphthalene were added. Then 92.8 ml (1.2 mole) of methylsulphonyl chloride were dropwise added with stirring and the temperature was allowed to rise to 60° C. Stirring was continued for 30 min and the reaction mixture poured into a mixture of 2 kg of ice and water to reach a temperature of 5° C., which temperature was suited for effecting diazotisation.

45 Diazotisation of o-aminobenzonitrile: 130 g (1.1 mole) of o-aminobenzonitrile were dissolved in 2 l of water whereto 275 ml of concentrated hydrochloric acid were added at 50° C. This solution was cooled to 0° C. Diazotisation was effected by dropwise addition of a solution of 79.35 g (1.15 mole) of sodium nitrite dissolved in 200 ml of water at 0° C. The reaction mixture was stirred at 0° C. for 30 min.

50 The azo-coupling proceeded at 5° C. by adding the diazonium salt solution with stirring to the solution of 1-methylsulphonylamino-7-sulpho-naphthalene in pyridine. Stirring was continued and 400 ml of concentrated hydrochloric acid were added.

55 60 The precipitate was suction-filtered, washed trice each time with 500 ml of 10% by weight aqueous sodium chloride solution and dried. Yield: 395 g (sodium chloride content: 25% by weight).

(b)  
1-Methylsulphonylamino-4-(2-cyanophenylazo)-7-chlorosulphonyl-naphthalene (compound P)

430 g of the reaction product Va were stirred in 2 l of 1,2-dichloroethane and heated to remove the residual water. The mixture was cooled to 40° C. whereupon 100 ml of N-methylpyrrolidinone were added. Then 300 ml of phosphorous oxychloride were added dropwise till the temperature reached 50° C. Stirring was continued at 50° C. for 2 h. After cooling over night, the precipitate was suction-filtered and washed trice each time with 300 ml of methylene chloride. After drying, the precipitate was stirred in 2 l of water, separated again and dried. Yield: 163 g.

(c)  
1-methylsulphonylamino-4-(2-cyano-phenylazo)-7-(p-sulphino-phenylsulphonyl)-naphthalene (compound Q)

To a solution of 52.5 g of p-aminobenzene sulphonic acid and 96 g of potassium carbonate in 850 ml of water first 1 l of acetone was added and then portionwise 157 g of compound P with stirring. Thereupon, the mixture was stirred for 1 h, poured into 2.5 l of water and acidified with 100 ml of concentrated hydrochloric acid. The precipitate formed was sucked off, washed with methanol and dried. Yield: 160 g.

We claim:

1. A process for the production of a multicolour dye image by dye diffusion transfer comprising the steps of:

- (1) image-wise multicolour photo-exposing a photographic multilayer multicolour material, which contains at least one developing agent and which is free from development nuclei for the silver complex diffusion transfer process and comprises a support carrying at least two differently spectrally sensitized alkali-permeable silver halide hydrophilic colloid emulsion layers each of which contains in operative contact therewith or therein a different non-diffusing dye or dye precursor compound that when contacted with an aqueous alkaline liquid remains immobile in an alkali-permeable colloid layer and is capable of being reduced by the said developing agent at a rate slower than the reduction of image-wise developable silver halide and in reduced state under alkaline conditions is capable of releasing a diffusible dye or dye precursor moiety, and
- (2) applying an alkaline liquid to said photoexposed material, thus effecting development of the photo-exposed material and image-wise diffusion-transfer therefrom of said diffusible dye or dye precursor moiety to a receptor layer,

characterized in that said alkaline liquid during development contains a silver halide solvent which is a thiosulphate, a thiocyanate, a thiosugar, a thioether acid or an active methylene compound having the methylene group linked directly to sulphonyl groups, and said solvent is present in an amount sufficient to form an alkali-soluble and reducible silver complex compound.

2. A process according to claim 1, characterized in that the non-diffusing dye or dye precursor compound is a ballasted compound capable of undergoing an electron-accepting nucleophilic displacement reaction separating hereby in alkaline medium a diffusible dye or dye precursor moiety.

3. A process according to claim 1, characterized in that the non-diffusing dye or dye precursor compound

is a ballasted compound capable of being split by reduction under alkaline conditions into a ballasted quinone-methide compound and a diffusible dye or dye precursor moiety.

4. A process according to claim 1, characterized in that the said developing agent(s) is (are) acting as (an) electron-transfer agent(s), and is (are) used together with (an) electron donor(s) which is unoxidized form are capable of reducing said non-diffusible dye or dye precursor compound, the said developing agent(s) being better silver halide reducing agents under the applied conditions of processing than the electron donors and providing by electron transfer an image-wise pattern of oxidized electron donor compounds corresponding to the developed silver halide.

5. A process according to claim 4, characterized in that said electron donor is present in non-diffusible state in each silver halide emulsion layer containing said different non-diffusing dye or dye precursor compound.

6. A process according to claim 4, characterized in that the electron transfer agent is a 3-pyrrolidinone compound and the electron donor is ascorbyl palmitate.

7. A process according to claim 1, characterized in that the photographic multicolour material comprises a support, which is coated in successive order with

- (1) a red-sensitive silver halide emulsion layer containing a non-diffusing dye compound comprising a diffusible moiety providing a cyan image dye and a non-diffusing electron donor compound,
- (2) a hydrophilic colloid interlayer containing a diffusible electron transfer agent,
- (3) a green-sensitive silver halide emulsion layer containing a non-diffusing dye compound comprising a diffusible moiety providing a magenta image dye and a non-diffusing electron donor compound,
- (4) a hydrophilic colloid interlayer containing a diffusible electron transfer agent,
- (5) a blue-sensitive silver halide emulsion layer containing a non-diffusing dye compound comprising a diffusible moiety providing a yellow image dye and a non-diffusing electron donor compound, and
- (6) a protective hydrophilic colloid layer containing a diffusible electron transfer agent.

8. A process according to claim 1, characterized in that said alkaline liquid contains a saturated, aliphatic or alicyclic amino alcohol having from 2 to 10 carbon atoms and at least two hydroxy groups, dimethylformamide, N-methyl-2-pyrrolidinone and/or an aliphatic or cycloaliphatic hydroxy compound that is not completely miscible with water at 20° C.

9. A process for the production of a multicolour dye image by dye diffusion transfer comprising the steps of:

- (1) image-wise multicolour photo-exposing a photographic multilayer multicolour material, which contains at least one developing agent and which is free from development nuclei for the silver complex diffusion transfer process and comprises a support carrying at least two differently spectrally sensitized alkali-permeable silver halide hydrophilic colloid emulsion layers each of which contains in operative contact therewith or therein a different non-diffusing dye or dye precursor compound that when contacted with an aqueous alkaline liquid remains immobile in an alkali-permeable colloid layer and is capable of being reduced by the said developing agent at a rate slower than the reduction of image-wise developable silver halide and in reduced state under alkaline conditions is

capable of releasing a diffusible dye or dye precursor moiety, and

(2) applying an alkaline liquid to said photoexposed material, thus effecting development of the photoexposed material and image-wise diffusion-transfer therefrom of said diffusible dye or dye precursor moiety to a receptor layer,

characterized in that said alkaline liquid during development contains a silver halide solvent which is set free in said alkaline aqueous liquid from a precursor compound incorporated in the photographic material corresponding to the following general formula:



wherein:

X represents the atoms necessary to complete a benzene or naphthalene nucleus,  
 Y is hydroxy or a substituent that upon hydrolysis provides hydroxy,  
 PHOTO represents a silver halide solvent moiety,  
 BALLAST is a ballasting group rendering said compound less diffusible in a water-permeable hydrophilic colloid layer than it would be without said group, and  
 n is 1 or 2;  
 and said solvent is present in an amount sufficient to form an alkali-soluble and reducible silver complex compound.

\* \* \* \* \*

25

30

35

40

45

50

55

60

65